

(No Model.)

P. WENZEL.

ENAMELED SLATE.

No. 333,578.

Patented Jan. 5, 1886.



Philip Wenzel

Attest:

John G. Hinkel Jr.  
Am. J. Fayers.

Inventor:

Foster & Freeman  
Attest

# UNITED STATES PATENT OFFICE.

PHILIPP WENZEL, OF MENTZ, GERMANY.

## ENAMELED SLATE.

SPECIFICATION forming part of Letters Patent No. 333,578, dated January 5, 1886.

Application filed April 29, 1885. Serial No. 163,903. (No model.) Patented in Germany October 7, 1884, No. 29,267.

*To all whom it may concern:*

Be it known that I, PHILIPP WENZEL, a citizen of the German Empire, residing at Mentz, Germany, have invented certain new and useful Improvements in Slates, of which the following is a specification.

My invention relates to writing-slates, and has for its object to produce an improved writing-slate having a white surface upon a practically indestructible base that shall be cheap, durable, and practicable; and to these ends my invention consists in a sheet metal coated or covered with enamel on one or both sides, the enamel being properly prepared to receive the marks from an ordinary black or other lead pencil.

It has been found that a slate with a white surface upon which black or other colored lines can be easily and accurately drawn is a great desideratum, being much better for the eyes than a black or dark slate upon which white lines or marks must be made. Moreover, a slate having a practically indestructible body or base, if properly made, has many advantages over the slates in common use. Many attempts have been made to overcome these objections and to produce a practically indestructible slate having a white writing-surface, as by covering a sheet of tin with white paint; but these have been found to lack the quality of durability, as well as failing to properly receive the marks made thereon, and to allow of their erasure without injuring the surface of the slate. White slates have also been made of glass, porcelain, marble, and the like; but these are expensive and easily destroyed. Paper and wooden slates have been made in a variety of colors by applying paints or coloring-matter thereto, and it has been proposed to make slates of celluloid plates treated with emery-powder and reinforced; but these have not proved efficient or durable, as the moisture generally used to erase the marks thereon speedily injures or destroys the body of the slate.

The object of my invention is to overcome all these difficulties, and I accomplish this object by constructing slates in a manner more particularly pointed out hereinafter.

I use a metallic base of some sheet metal, preferably iron, and this may be quite thin, and

consequently cheap. The surfaces of the sheet metal are first thoroughly cleaned and an enamel applied thereto in any convenient manner, as by mixing the enamel-powder in the form of a paste, which is spread over the surfaces of the metal plate and allowed to dry. The enamel may be of various kinds; but to produce a fine clear white surface I find that an enamel composed, essentially, of silicious materials having some metallic oxides or earths mixed therewith are cheap, durable, and practicable. The enamel having been properly applied to the surfaces of the metal base, it is placed into a suitable muffle-furnace wherein the temperature is raised to such a degree that the enamel melts and forms a thin even coating all over the plate, and at the same time it adheres closely to the plate, so that it is not liable to crack or peel off or otherwise become uneven. Upon removing the plate from the muffle-furnace and cooling the same, the enameled surface is found to be too smooth to properly take the lead or other substance from the pencil and to receive and retain the marks, and to properly prepare the surface for that purpose I remove the exterior glaze or surface of the enamel, or roughen or mat the same by immersing it in a bath of some proper acid—as hydrofluoric or equivalent acid—acting destructively upon the enamel, where it remains a sufficient time to allow the acid to “bite” the enameled or glazed surface to produce the desired toothed or matted condition to best receive and retain the marks. In some cases this condition of the surface may be produced by abrasion, as by a sand-blast; but I have found the acid bath most convenient and satisfactory. The surfaces having been properly prepared, the material may be cut to any desired size or shape and framed in any of the well-known ways. In this way I am enabled to produce a slate having a white surface on a very thin metallic base, that is light, cheap, and practically indestructible, and one on which the ordinary black-lead pencils may be freely and conveniently used to produce good, sound, and unbroken black or colored lines, and these lines may be easily and thoroughly erased without leaving any traces on the surface or injury to the enamel.

In the accompanying drawing, forming a

part of this specification, I have shown a representation of my invention as embodied in a slate having a frame of ordinary shape and construction, the surface of the slate being 5 white with black lines thereon.

It is understood that the sheet metal may be covered or coated with the enamel surface on one or both sides, as desired.

I do not desire to limit myself to the precise details set forth above, as they may be varied without departing from the spirit of 10 my invention.

I have used the word "white" as applied to the color of the slate in a relative sense, as 15 compared with the dark mark of the pencil.

What I claim as my invention is—

1. A writing-slate consisting of a metal body coated or covered with enamel and having a white surface, substantially as described.

2. A writing-slate consisting of a sheet- 20 metal body coated or covered with enamel, the glaze of which is roughened or matted to present a white writing-surface, substantially as described.

3. A writing-slate consisting of a thin sheet- 25 iron base coated or covered with a white silicious enamel, the surface of which is bitten or roughened with acid, to produce a proper writing surface.

In testimony whereof I have signed my 30 name to this specification in the presence of two subscribing witnesses.

PHILIPP WENZEL. [L. S.]

Witnesses:

JOH. A. HOUG,  
Jos. SCOTT.